

April 24, 1956

A. M. TALBOT

2,743,175

PRECISION CASTING ALLOY

Filed Jan. 27, 1953

2 Sheets-Sheet 1



Fig. 1.

INVENTOR.

ALBERT MCCOY TALBOT

BY G. R. Miller  
ATTORNEY

April 24, 1956

A. M. TALBOT

2,743,175

PRECISION CASTING ALLOY

Filed Jan. 27, 1953

2 Sheets-Sheet 2



*Fig. 2.*



*Fig. 3.*

INVENTOR.

ALBERT McCORY TALBOT

BY *G. R. Weller*

ATTORNEY

1

2,743,175

## PRECISION CASTING ALLOY

Albert M. Talbot, Fair Haven, N. J., assignor to The International Nickel Company, Inc., New York, N. Y., a corporation of Delaware

Application January 27, 1953, Serial No. 333,523

9 Claims. (Cl. 75—128)

The present invention relates to improved high temperature heat- and stress-resisting precision cast articles suitable for use at elevated temperatures in power plant units of aircraft gas turbine engines, turbojet engines, and the like and to special heat- and stress-resisting nickel-chromium-iron alloys substantially free from the strategically scarce metals cobalt, columbium and tungsten.

In recent years the art has been earnestly endeavoring to obtain heat- and stress-resisting cast alloys capable of withstanding high stresses at high temperatures in the range from about 1200° F. to about 1800° F., particularly alloys suitable for use as blading material in aircraft gas turbine engines, turbojet engines, etc. A major difficulty which has confronted the art has been the modern trend to design aircraft engines to operate at higher and higher temperatures. At the higher operating temperatures, i. e., temperatures in excess of 1350° F. and even in excess of 1500° F., the service life of the alloys is greatly reduced. To be assured of a service life of even a few hundred hours, it has been necessary to employ alloys containing substantial amounts of strategically scarce elements, such as cobalt, columbium and/or tungsten, particularly large amounts of cobalt. Cobalt-base alloys containing either columbium or tungsten or both have been found effective in meeting the rigorous operating requirements of aircraft gas turbine engines, turbojet engines, and the like. However, the aforementioned elements are usually found in countries which are not completely accessible during times of international emergency. When such emergency conditions prevail, which interfere with the obtaining of such strategically scarce elements as cobalt, columbium and tungsten, etc., other alloying materials must be resorted to in the making of heat-resisting alloys, particularly alloying materials which are readily available. In cognizance of this situation, many attempts have been made to employ substitute alloys low in or substantially free from strategically scarce elements. However, many of the substitute non-strategic alloys employed have not been generally satisfactory in that these alloys did not always meet the high temperature strength and creep properties required at the high service temperatures and also did not usually meet the service life usually obtained by the cobalt-base alloys.

In producing high temperature articles, it has usually been necessary to produce them by mechanical working operations rather than by casting the alloys directly into their final shape. Many of the alloys which possessed the required high temperature properties, usually very high in strategically scarce elements, did not have the required properties in the as-cast condition to permit their use as castings. Also, some of the alloys which contained large amounts of other alloying materials for the purpose of

2

imparting improved resistance to deformation at elevated temperatures were difficult to hot work into articles of the desired shape for service. Thus, the use of mechanical working operations for producing high temperature articles from such alloys greatly increased the cost of the articles. This was particularly true when producing wrought articles having somewhat complicated shapes which usually also required many finishing operations in producing the final shape. Moreover, in addition to the increased cost due to the mechanical working operation, there was also the problem of increased cost in producing the final article by machining, grinding, polishing, etc. A further disadvantage of wrought articles was the necessity in many instances of employing special high temperature heat treatments in order to develop the required high temperature properties. Since in many cases the special heat treatments were applied to the finished article prior to use, many of the articles were subject to twisting, warping, etc., due to the thermal stresses set up during heat treatment and, therefore, had to be rejected or discarded. In view of the foregoing, there has been a demand for alloys suitable for producing articles having complicated and intricate shapes for turbine blades, turbine buckets, etc., by employing precision casting methods which are also sometimes referred to as "lost-wax" processes. Since many of the known wrought alloys did not have the necessary casting properties required for precision casting, a demand has existed for special cast alloys having high temperature properties comparable to those of wrought alloys and also having the required precision casting properties. While many cast alloys have been developed meeting high temperature requirements, these alloys did not always have the required casting properties in that some of the alloying elements employed oxidized easily or formed scum during melting which appeared to interfere with the fidelity of precision castings. Furthermore, many of the suitable precision casting alloys required the presence of substantial amounts of the strategically scarce elements mentioned hereinbefore and/or required special heat treatments in order to develop the desired high temperature properties. Although many attempts were made to overcome the foregoing difficulties and other difficulties and disadvantages, none, as far as I am aware, was entirely successful when carried into practice commercially on an industrial scale.

I have now discovered an improved high temperature heat- and stress-resisting precision cast article comprised of an alloy which is substantially free from the strategically scarce alloying elements cobalt, columbium and tungsten, which possesses the requisite casting properties demanded by precision casting methods and which has the required high temperature properties, including heat resistance, stress resistance, creep resistance, etc.

It is an object of the invention to provide an improved non-strategic, nickel-chromium-iron precision cast article for use at high temperatures in gas turbines, turbojet engines, and the like.

Another object of the invention is to provide a special cobalt-free, columbium-free, tungsten-free, nickel-chromium-iron, heat- and stress-resisting article for use at high temperatures in gas turbines, turbojet engines, and the like, made of an alloy containing a novel and synergistic combination of relatively non-strategic elements within critical ranges.

It is a further object of the present invention to provide an improved casting alloy free from strategically scarce elements and having high temperature properties sub-

## 3

stantially comparable to cast alloys containing substantial amounts of strategically scarce elements.

The invention also contemplates providing an improved non-strategic, nickel-chromium-iron alloy for use at high temperatures, said alloy being characterized by good heat- and stress-resisting properties at high temperatures.

Other objects and advantages will become apparent from the following description taken in conjunction with the accompanying drawing in which:

Figure 1 depicts comparative rupture life curves which illustrate the synergistic effects of the critical combination of elements employed in the novel alloy.

Fig. 2 illustrates curves showing the 100-hour and 1000-hour rupture strengths of an alloy within the scope of the invention.

Fig. 3 depicts curves illustrating stress rupture life properties of the alloy contemplated by the invention at various high temperatures.

Generally speaking, the present invention contemplates novel high temperature, heat- and stress-resisting cast articles adapted for use in aircraft gas turbines, turbojet engines, and the like, comprising a special nickel-chromium-iron alloy substantially free from the strategically scarce elements, cobalt, columbium and/or tungsten. The present invention is based on the discovery that nickel-chromium-iron alloys having improved high temperature strength properties can be produced by incorporating in the alloy critical and controlled amounts of the relatively non-strategic alloying elements molybdenum, boron, and carbon. The alloy employed in producing articles in accordance with the invention is amenable to precision casting methods and is particularly applicable to the fabrication by precision casting methods of cast articles of complicated shape, including aircraft turbine blades, for service at high temperatures under high stresses in gas turbines, turbojet engines, etc. The alloy is also amenable to fabrication by powder metallurgy. In general, the alloy contains as critical and essential elements about 19% to 50% nickel, 18% to 30% chromium, 8% to 12% molybdenum, 0.03% to 0.8% boron, 0.5% to 1.5% carbon and the balance essentially iron which constitutes at least about 10% but may be as high as about 55% of the alloy. In producing cast nickel-chromium-iron articles having high fracture life at elevated temperatures comparable to cast articles made of alloys containing substantial amounts of strategically scarce elements, it is preferred that the alloy composition of the articles be maintained within the range of about 20% to 40% nickel, 20% to 30% chromium, 8% to 10% molybdenum, 0.05% to 0.3% boron and 0.6% to 1.2% carbon. The balance of the preferred alloy composition is essentially iron which constitutes about 15% to 50% of the alloy.

It is an essential feature of the invention that the amounts of nickel, chromium and iron be correctly proportioned within the ranges specified hereinbefore and be employed in combination with critical and controlled amounts of molybdenum, boron and carbon. It has been found that the changes in the amount of nickel have a more important effect upon the properties than corresponding changes in the amount of chromium. Increasing the nickel content to about 35% results in optimum rupture life properties which fall off rapidly when the nickel content of the alloy exceeds 50%. For this reason, the maximum nickel content of the alloys contemplated by the invention is about 50%. Too low a nickel content endangers the austenite stability and the high properties of the alloys contemplated by the invention. For this reason, the nickel content should not be less than about 20% or 19%. Stress rupture tests conducted on the novel alloy at elevated temperatures have indicated that the elements molybdenum, boron and carbon are critical and are synergistic in effecting the improved results provided by the invention when the three elements are controlled within the specified ranges. When one

## 4

or more of the elements molybdenum, boron and carbon are absent from the cast alloy or are not within the ranges prescribed hereinbefore, the final properties of the alloy are greatly affected in that the results contemplated by the invention are not obtained.

It is preferred when producing articles made of alloys within the foregoing ranges of composition by precision casting that boron be employed in amounts ranging from about 0.10% to about 0.3%. Silicon may be present in the alloy up to about 2% but is not essential. However it is desirable that silicon be present as it improves the castability of the alloy. Manganese likewise may be optionally employed up to about 3% in producing the alloy provided by the invention. When the two foregoing elements are employed in the alloy, they are usually present in amounts ranging from about 0.1% to 2% silicon and from about 0.1% to 3% manganese. It is preferred to employ manganese in amounts ranging from about 1.5% to 2%. In this range, manganese, is effective in improving the castability of the alloy. The expression "the balance" or "the balance essentially" iron does not exclude silicon and manganese in the foregoing amounts. Other elements may be present in the alloy in incidental amounts without deleteriously affecting the properties of the alloy. Such incidental elements may be present as the result of scrap contamination, as a result of the use of master addition alloys, from the use of deoxidizers, degasifiers, purifiers and the like, during processing, etc. The incidental elements which may be present in the alloy include up to about 0.1% aluminum, up to about 0.03% magnesium, up to about 0.03% calcium, up to about 0.1% copper, etc. It is to be understood that certain gases may be picked up from the atmosphere during melting and as a result are unavoidably present in small amounts. Thus, nitrogen may be picked up in this way and may be present in amounts up to about 0.15% and is not detrimental even when intentionally added in amounts up to about 0.2%. However, the presence of nitrogen in greater amounts leads to porosity of the casting. The rare earth elements, lanthanum and cerium, may be present in amounts of less than about 0.1% to counteract the detrimental effects of any sulfur present and to improve the surface condition of castings. The total per cent of all the incidental elements together should not exceed about one per cent. Impurities, such as sulfur and phosphorus, should be kept as low as is commercially feasible. While the alloy is characterized as being cobalt-free, small amounts of cobalt may be present in incidental amounts up to about one per cent and may be introduced into the alloy incidental to the addition of other elements. For example, cobalt may be introduced in the alloy along with commercial nickel which often contains small amounts of cobalt up to about 1% or 2% or even more. Likewise, small amounts of titanium may be present incidental to the manufacture of the alloy.

A composition range which has been found to be particularly adaptable for commercial use comprises about 30% to 34% nickel, 23% to 27% chromium, 8% to 10% molybdenum, 0.05% to 0.3% boron, 0.6% to 1% carbon, up to 2% manganese, up to 1.5% silicon and the balance essentially iron, including the usual amounts of incidental elements and impurities. In the foregoing composition it is preferred that the boron content be at least 0.10%. A nominal composition of such an alloy would comprise about 32% nickel, about 25% chromium, about 9% molybdenum, about 0.8% carbon, about 0.15% boron, about 1.5% manganese, about 0.4% silicon and the balance essentially iron.

In evaluating heat resistant alloys for use in gas turbine engines, turbojet engines and the like, high temperature rupture tests are usually employed. One such test, which is usually referred to by those skilled in the art as a stress rupture test, comprises subjecting an alloy specimen to a given stress at an elevated temperature and maintaining the stress until the alloy fractures. The time

it takes for the alloy to fracture under the given stress is taken as an indication of how the alloy might behave under operating conditions in actual service. For example, a test commonly employed in evaluating stress rupture life of a cast alloy at elevated temperatures comprises subjecting the alloy specimen to a high stress, e. g., a stress of about 28,000 pounds per square inch (p. s. i.), at a given temperature, for example, about 1350° F. Data obtained from the foregoing type of test permits determining the 100-hour or 1000-hour rupture life of the alloy, which is the stress which will produce rupture in 100 hours or 1000 hours, respectively, at the temperature of test. A cast alloy is usually considered adequate when it has a 100-hour rupture life at a temperature of about 1350° F. when subjected to a rupture stress of about 34,000 p. s. i. The alloy produced in accordance with the invention generally has a 100-hour rupture life at about 1350° F. when subjected to a rupture stress of at least about 37,000 or 38,000 p. s. i. and may attain as high as 46,000 p. s. i. under certain conditions.

For the purpose of giving those skilled in the art a better understanding of the invention and a better appreciation of the advantages of the invention, the following illustrative examples are given:

*Example I*

An alloy embodying the present invention was produced having the following composition:

| Alloy No. | Per cent Ni | Per cent Cr | Per cent Mo | Per cent B | Per cent C | Per cent Mn | Per cent Si | Per cent Fe |
|-----------|-------------|-------------|-------------|------------|------------|-------------|-------------|-------------|
| 1-----    | 35          | 28          | 9           | 0.19       | 1.14       | 0.5         | 0.5         | Bal.        |

The procedure followed in producing the aforementioned alloy comprised melting proper proportions of alloy ingredients, such as ingot iron, metallic nickel, high-carbon ferro-chrome, ferro-molybdenum, ferro-manganese and ferro-boron, in a high-frequency induction furnace. All of the foregoing materials, except ferro-boron, were melted and the melt deoxidized with either ferro-silicon or silico-manganese and wherever necessary carburized with washed pig iron. The boron addition was made immediately before casting the metal which was cast into sand molds in the shape of miniature pigs suitable for remelting in an indirect arc furnace customarily used for precision casting. The miniature pigs were remelted in the indirect arc furnace and poured into an investment mold produced by the "lost-wax" process to produce precision cast test bars measuring about 0.25 inch in diameter and having a one-inch gauge length.

The foregoing alloy was subjected in the as-cast condition to a stress rupture test at 1350° F. at various stresses. The following schedule sets forth the results and demonstrates the markedly high rupture lives exhibited by this alloy.

| Stress, p. s. i. | Rupture Life, hours |
|------------------|---------------------|
| 35,000-----      | 616                 |
| 40,000-----      | 249                 |

The alloy after fracture under the foregoing test conditions exhibited a ductility of about 6% to 9% measured as per cent elongation over a gauge length of one inch. This alloy in the as-cast condition is also capable of withstanding a high stress of about 44,000 p. s. i. at 1350° F. for 100 hours before rupture occurs. Likewise, this alloy would withstand a stress of 28,000 p. s. i. for about 3,500 hours at a temperature of about 1350° F.

*Example II*

Other embodiments of the present invention which have given good results are illustrated by the following alloys:

| Alloy No. | Per cent Ni | Per cent Cr | Per cent Mo | Per cent B | Per cent C | Per cent Mn | Per cent Si | Per cent Fe |
|-----------|-------------|-------------|-------------|------------|------------|-------------|-------------|-------------|
| 2-----    | 35.4        | 26.1        | 8.1         | 0.12       | 0.93       | 1.52        | 0.42        | Bal.        |
| 3-----    | 34.7        | 27.4        | 8.1         | 0.13       | 0.93       | 1.66        | 0.48        | Bal.        |
| 4-----    | 35.4        | 26.0        | 8.1         | 0.18       | 0.90       | 1.52        | 0.42        | Bal.        |
| 5-----    | 35          | 28          | 8           | 0.18       | 0.95       | 2           | 0.4         | Bal.        |
| 6-----    | 35          | 28          | 8           | 0.13       | 0.98       | 2           | 0.4         | Bal.        |
| 7-----    | 35          | 28          | 8           | 0.21       | 0.96       | 2           | 0.4         | Bal.        |
| 8-----    | 35          | 28          | 8           | 0.24       | 0.95       | 2           | 0.4         | Bal.        |
| 9-----    | 35          | 28          | 9.2         | 0.24       | 0.53       | 0.42        | 0.47        | Bal.        |
| 10-----   | 34.9        | 28.1        | 9.3         | 0.27       | 0.58       | 0.41        | 0.46        | Bal.        |
| 11-----   | 35          | 28          | 9           | 0.1        | 0.62       | 0.4         | 0.5         | Bal.        |
| 12-----   | 35          | 28          | 9.2         | 0.12       | 0.72       | 0.42        | 0.50        | Bal.        |
| 13-----   | 35.6        | 27.5        | 9.1         | 0.17       | 0.88       | 0.44        | 0.63        | Bal.        |
| 14-----   | 35.5        | 27.3        | 9.3         | 0.17       | 1.02       | 1.48        | 0.48        | Bal.        |
| 15-----   | 35          | 28          | 9           | 0.1        | 1.11       | 0.4         | 0.5         | Bal.        |
| 16-----   | 35          | 28          | 11.8        | 0.08       | 0.98       | 0.4         | 0.5         | Bal.        |
| 17-----   | 35          | 28          | 11.5        | 0.10       | 0.93       | 0.4         | 0.5         | Bal.        |

<sup>1</sup> Both Alloy No. 11 and Alloy No. 15 contained about 0.2% nitrogen.

In preparing and casting the foregoing alloys, the procedure described for Example I was employed. It will be noted from the foregoing table that the compositions of the nickel-chromium-iron alloys comprise about 35% nickel, about 26% to 28% chromium and the essential critical elements molybdenum, boron and carbon in amounts ranging from 8% to about 12% molybdenum, from about 0.08% to about 0.3% boron and from about 0.5% to about 1.1% carbon, the balance of the alloy being essentially iron including such other ingredients as manganese, silicon, nitrogen, etc.

The foregoing alloys, when subjected in the as-cast condition to a stress rupture test at 1350° F. at various stresses gave the following rupture lives:

| Alloy No. | Rupture Life at 1350° F. in hours under stress of- |                 |                 |
|-----------|----------------------------------------------------|-----------------|-----------------|
|           | 35,000 p. s. i.                                    | 40,000 p. s. i. | 45,000 p. s. i. |
| 2-----    |                                                    | 98              | 28              |
| 3-----    |                                                    | 71              | 33              |
| 4-----    | 242                                                | 82              |                 |
| 5-----    |                                                    | 143             | 61              |
| 6-----    |                                                    | 122             | 25              |
| 7-----    |                                                    | 105             | 60              |
| 8-----    |                                                    | 78              | 24              |
| 9-----    | 1655                                               |                 |                 |
| 10-----   | 147                                                | 72              |                 |
| 11-----   | 215                                                | 93              |                 |
| 12-----   | 613                                                | 195             |                 |
| 13-----   | 583                                                | 143             |                 |
| 14-----   | 442                                                | 119             |                 |
| 15-----   | 472                                                | 157             |                 |
| 16-----   |                                                    | 67              |                 |
| 17-----   | 180                                                | 122             |                 |

<sup>1</sup> Under rupture stress of 28,000 p. s. i.

<sup>2</sup> Under rupture stress of 33,000 p. s. i.; extrapolated rupture life under stress of 28,000 p. s. i. is about 1300 hours.

<sup>3</sup> Under rupture stress of 33,000 p. s. i.; under rupture stress of 37,000 p. s. i., rupture life is 261 hours.

The foregoing alloys after fracture under the aforementioned test conditions exhibited ductility values ranging from about 4% to 17% measured as per cent elongation over a gauge length of one inch.

The stress to give a rupture life of 100 hours at 1350° F. for each of the above alloys is given in the following table:

| Alloy No. | 100-hour Rupture Stress in p. s. i. |
|-----------|-------------------------------------|
| 2-----    | 40,000                              |
| 3-----    | 38,000                              |
| 4-----    | 39,000                              |
| 5-----    | 42,000                              |
| 6-----    | 41,000                              |
| 7-----    | 40,000                              |
| 8-----    | 39,000                              |
| 9-----    | 37,000                              |
| 10-----   | 38,000                              |
| 11-----   | 39,000                              |
| 12-----   | 45,000                              |
| 13-----   | 42,000                              |
| 14-----   | 41,000                              |
| 15-----   | 42,000                              |
| 16-----   | 43,000                              |
| 17-----   |                                     |

## 7 Example III

Still other illustrative alloys within the scope of the invention and produced in accordance with the procedure of Example I are as follows:

| Alloy No. | Per cent Ni | Per cent Cr | Per cent Mo | Per cent B | Per cent C | Per cent Mn | Per cent Si | Per cent Fe |
|-----------|-------------|-------------|-------------|------------|------------|-------------|-------------|-------------|
| 18        | 34.93       | 20.03       | 8.00        | 0.11       | 0.80       | 1.56        | 0.45        | Bal.        |
| 19        | 30.13       | 25.85       | 8.60        | 0.11       | 0.78       | 1.28        | 0.42        | Bal.        |
| 20        | 24.60       | 27.50       | 8.96        | 0.12       | 0.81       | 1.14        | 0.49        | Bal.        |
| 21        | 19.83       | 27.69       | 9.24        | 0.18       | 0.91       | 1.19        | 0.39        | Bal.        |

The foregoing alloys were subjected in the as-cast condition to a stress rupture test at 1350° F. and at 1500° F. As a result of this test the following high rupture lives at stresses of 35,000 p. s. i. and 20,000 p. s. i., respectively, were obtained:

| Alloy No. | Rupture Life in hours—            |                                   |
|-----------|-----------------------------------|-----------------------------------|
|           | at 1350° F. under 35,000 p. s. i. | at 1500° F. under 20,000 p. s. i. |
| 18        | 435                               | 402                               |
| 19        | 539                               | 385                               |
| 20        | 500                               | 181                               |
| 21        | 185                               | 99                                |

The ductility of the foregoing alloys after fracture at 1350° F. and a rupture stress of 35,000 p. s. i. average about 18% while the ductility after fracture at 1500° F. and a rupture stress of 20,000 p. s. i. averaged about 20.5%.

## 8 Example IV

Other data illustrating the rupture life of the as-cast alloys within the scope of the present invention at 1500° F. and higher is set forth in the following schedule:

| Alloy No. | Temperature, ° F. | Stress, p. s. i. | Rupture Life, hours |
|-----------|-------------------|------------------|---------------------|
| 2         | 1500              | 25,000           | 75                  |
| 22        | 1500              | 25,000           | 58                  |
| 22        | 1500              | 24,000           | 122                 |
| 23        | 1500              | 24,000           | 107                 |
| 3         | 1500              | 22,000           | 213                 |
| 2         | 1500              | 22,000           | 45                  |
| 2         | 1500              | 20,000           | 278                 |
| 22        | 1500              | 20,000           | 180                 |
| 23        | 1500              | 18,000           | 460                 |
| 22        | 1500              | 18,000           | 350                 |
| 22        | 1500              | 16,000           | 1035                |
| 6         | 1650              | 13,000           | 115                 |
| 22        | 1650              | 13,000           | 104                 |
| 22        | 1650              | 11,000           | 330                 |
| 22        | 1650              | 10,000           | 592                 |
| 8         | 1800              | 10,000           | 16                  |
| 8         | 1800              | 8,000            | 35                  |
| 22        | 1800              | 6,000            | 250                 |

In the foregoing schedule, alloy No. 22 contained about 35% nickel, 29.5% chromium, 1.0% carbon, 2% manganese, 0.3% silicon, 8.8% molybdenum, 0.25% boron, and the balance essentially iron, and alloy No. 23 contained about 35% nickel, 28% chromium, 1.06% carbon, 2% manganese, 0.3% silicon, 9% molybdenum, 0.23% boron and the balance essentially iron.

Other nickel-chromium-iron alloy compositions which have been found to give the results provided by the invention are given in the following schedule:

| Alloy No. | Per cent Ni | Per cent Cr | Per cent Mo | Per cent B | Per cent C | Per cent Mn | Per cent Si | Per cent Fe |
|-----------|-------------|-------------|-------------|------------|------------|-------------|-------------|-------------|
| 24        | 35          | 28          | 11.5        | 0.77       | 0.94       | 0.4         | 0.5         | Bal.        |
| 25        | 48.4        | 26.7        | 9.1         | 0.10       | 1.05       | 1.7         | 0.5         | Bal.        |

Alloy No. 24, which contained high molybdenum and high boron contents (11.5% Mo and 0.77% B), exhibited a

high 100-hour rupture stress of 46,000 p. s. i. at a temperature of 1350° F. while alloy No. 25, which had a high nickel content of 48.4%, exhibited a high rupture life of 1453 hours under a stress of 28,000 p. s. i. at 1350° F.

For the purpose of better illustrating the advantages of the invention, a series of comparative tests were conducted with a group of alloys having compositions outside the scope of the invention. The compositions of these alloys are illustrated in the following schedule:

| Alloy No. | Per cent Ni | Per cent Cr | Per cent Mo | Per cent B | Per cent C | Per cent Mn | Per cent Si | Per cent Fe |
|-----------|-------------|-------------|-------------|------------|------------|-------------|-------------|-------------|
| A         | 35.3        | 15.2        | —           | —          | —          | 0.34        | 0.39        | 0.36        |
| B         | 49.2        | 26.6        | —           | —          | —          | 0.46        | 0.47        | 0.29        |
| C         | 34.8        | 27.0        | —           | —          | —          | 0.35        | 0.46        | 0.29        |
| D         | 50          | 28          | —           | —          | —          | 1.05        | 0.5         | 0.3         |
| E         | 42.7        | 26.6        | 9           | —          | —          | 0.38        | 1.94        | 0.3         |
| F         | 45.4        | 26.8        | —           | 0.11       | —          | 0.52        | 0.53        | 0.3         |
| G         | 35          | 28          | —           | —          | —          | 1.11        | 0.4         | 0.3         |
| H         | 35          | 28          | —           | —          | —          | 0.84        | 0.4         | 0.6         |
| I         | 35.7        | 25.6        | 8.7         | —          | —          | 0.34        | 0.30        | 0.65        |
| J         | 35          | 28          | —           | —          | —          | 1.80        | 0.4         | 0.6         |
| K         | 34.9        | 28.2        | 4.3         | 0.23       | —          | 0.45        | 0.41        | 0.55        |
| L         | 35          | 15          | 9           | 0.067      | —          | 0.44        | 2           | 0.4         |
| M         | 50          | 28          | 9.0         | 0.049      | —          | 0.28        | 2.06        | 0.3         |
| N         | 35          | 28          | 9.6         | —          | —          | 0.56        | 0.37        | 0.76        |
| O         | 34.3        | 27.6        | —           | —          | —          | 0.18        | 0.90        | 0.44        |
| P         | 35          | 20          | 9           | 0.082      | —          | 0.25        | 2           | 0.4         |
| Q         | 35          | 20          | 9           | 0.16       | —          | 0.26        | 2           | 0.4         |
| R         | 35.5        | 28          | 9           | 0.064      | —          | 0.28        | 2.2         | 0.3         |
| S         | 34.7        | 26.5        | 8.4         | 0.03       | —          | 0.41        | 0.44        | 0.32        |

The foregoing alloys were produced by procedures similar to those employed in producing the alloys described hereinbefore. The stress rupture results obtained on the foregoing alloys at elevated temperatures are as follows:

| Alloy No. | Rupture Life at 1350° F. in hours under stress of— |                 |                 | Stress in p. s. i. for 100-hour Life, 1350° F. |
|-----------|----------------------------------------------------|-----------------|-----------------|------------------------------------------------|
|           | 23,000 p. s. i.                                    | 28,000 p. s. i. | 33,000 p. s. i. |                                                |
| 40        | 6                                                  | 36              | 2.5             | 20,000                                         |
| A         | 6                                                  | 6               | 2.2             | —                                              |
| B         | 24                                                 | 28              | —               | —                                              |
| C         | 14                                                 | 19              | 3.2             | —                                              |
| D         | 28                                                 | 25              | —               | —                                              |
| E         | 26                                                 | 21              | —               | —                                              |
| F         | 168                                                | 196             | —               | —                                              |
| G         | 196                                                | 70              | —               | —                                              |
| H         | 94                                                 | 78              | 28,000          | —                                              |
| I         | 87                                                 | 36              | 27,000          | —                                              |
| J         | 343                                                | 108             | 28,000          | —                                              |
| K         | 610                                                | 78              | 27,000          | —                                              |
| L         | 137                                                | 56              | 29,000          | —                                              |
| M         | —                                                  | —               | —               | —                                              |
| N         | —                                                  | —               | —               | —                                              |
| O         | —                                                  | —               | —               | —                                              |
| P         | —                                                  | —               | —               | —                                              |
| Q         | —                                                  | —               | —               | —                                              |
| R         | —                                                  | —               | —               | —                                              |
| S         | —                                                  | —               | —               | —                                              |

<sup>1</sup> Under a stress of 20,000 p. s. i.

<sup>2</sup> Under a stress of 35,000 p. s. i.

It will be noted from the foregoing schedule that all of the alloys outside the scope of the invention had low stress rupture values and were markedly inferior to the alloys provided by the invention.

As has been stated hereinbefore, it is important in carrying out the invention that the alloy contain carbon, boron and molybdenum in order to obtain the desired improved properties in cast articles made of the alloy provided by the invention. The three elements cooperate to produce a synergistic effect in the relatively non-strategic cast alloy to produce good rupture life at elevated temperatures. This effect can be illustrated by Fig. 1 which compares the influence of carbon on the rupture life of alloys containing about 35% nickel, 28% chromium and both molybdenum and boron in proper amounts (curve A) with the influence of carbon in similar nickel-chromium alloys containing molybdenum but devoid of boron (curve B) or containing boron but devoid of molybdenum (curve C) or devoid of both boron and molybdenum (curve D). The curves depicted in Fig. 1 are based on rupture tests conducted under a stress of

28,000 p. s. i. at 1350° F. In Fig. 1, curves B, C and D show the inferior rupture lives which are obtained with varying carbon contents in alloys containing molybdenum but devoid of boron, containing boron but devoid of molybdenum and devoid of both molybdenum and boron, respectively, while curve A illustrates the markedly improved results which are obtained when synergistic proportions of carbon are present in accordance with the invention in the nickel-chromium alloys containing both molybdenum and boron in critical amounts. Thus, at a carbon level of 0.6%, the alloy devoid of both molybdenum and boron (curve D) would have an inferior stress rupture life of less than 25 hours, the alloy devoid of molybdenum but containing boron (curve C) would have an inferior stress rupture life of less than 50 hours, while the alloy containing molybdenum but devoid of boron (curve B) would have a low stress rupture life of close to 100 hours. In contradistinction, the alloy within the scope of the invention having the same carbon content of 0.6% would have the remarkably improved rupture life of over about 500 hours (curve A). Likewise, at a carbon level of 0.7%, it will also be noted from the curves of Fig. 1 that the alloy devoid of both molybdenum and boron (curve D) would have an inferior stress rupture life of less than 25 hours, the alloy devoid of molybdenum but containing boron (curve C) would have an inferior stress rupture life of less than 50 hours, while the alloy containing molybdenum but devoid of boron (curve B) would have a low stress rupture life of less than 150 hours. On the other hand, it will be noted that the alloy within the scope of the invention and having the same carbon level of 0.7% would have the remarkably high stress rupture life of over about 1000 hours (curve A). It will also be noted from Fig. 1 (curve A) that the carbon appears to have its most critical effect when it is present in the alloy provided by the invention in amounts above about 0.5%.

The importance of carbon as an essential element is also shown by the following schedule which illustrates the marked critical effect of carbon on the 100-hour rupture stress of the alloy at 1350° F.

| Alloy No. | Percent C | Rupture Stress at 1350° F. to give 100-hour life, p. s. i. |
|-----------|-----------|------------------------------------------------------------|
| T         | 0.20      | 29,000                                                     |
| U         | 0.29      | 30,000                                                     |
| S         | 0.41      | 29,000                                                     |
| 11        | 0.62      | 39,000                                                     |
| 3         | 0.93      | 38,000                                                     |
| 2         | 0.93      | 40,000                                                     |
| 6         | 0.98      | 41,000                                                     |
| 15        | 1.11      | 42,000                                                     |

All the alloys in the foregoing schedule contained, in addition to the specified amounts of carbon, approximately 35% nickel, approximately 28% chromium, about 8% to 9% molybdenum, about 0.08% to 0.13% boron and the balance essentially iron plus the usual incidental elements and impurities. It will be noted that the alloys containing above about 0.5% carbon exhibit marked improved 100-hour rupture stress of the order of 38,000 p. s. i. or better whereas the alloys containing less than about 0.5% carbon exhibit inferior rupture stress values of the order of 29,000 to 30,000 p. s. i.

Similar alloys having higher boron content, e. g., 0.16% to 0.27% boron, also show the critical effect of carbon on the 100-hour rupture stress of the alloy at 1350° F. as illustrated by the data in the following schedule:

| Alloy No. | Percent C | Rupture Stress at 1350° F. to give 100-hour life, p. s. i. |
|-----------|-----------|------------------------------------------------------------|
| Q         | 0.26      | 27,000                                                     |
| 9         | 0.53      | 37,000                                                     |
| 10        | 0.58      | 38,000                                                     |
| 13        | 0.86      | 42,000                                                     |

It will be noted from the foregoing schedule that alloys within the scope of the invention and containing above about 0.5% of carbon exhibit a 100-hour rupture stress value of at least about 37,000 p. s. i. On the other hand, when the carbon content is below about 0.5%, e. g., 0.26% carbon, the alloy exhibits a low 100-hour rupture stress value, e. g., 27,000 p. s. i.

The two foregoing schedules illustrate the marked critical effect which carbon has been found to exert in combination with the remainder of the composition in improving the 100-hour rupture life when it is present in the alloy provided by the present invention in amounts of about 0.5% carbon and higher. Likewise, similar data have indicated that the minimum content of boron should be 0.03% and the minimum content of molybdenum should be 8% in order to obtain the results provided by the invention.

The high temperature properties exhibited by the relatively non-strategic cast alloy provided by the invention compare very favorably with prior art cast alloys containing a large amount of such strategically scarce elements cobalt, columbium, and/or tungsten. For example, the following schedule compares the 100-hour and the 1000-hour rupture strengths (as stress in pounds per square inch) of the novel alloys at 1350° F. and 1500° F. with two prior art alloys referred to in the art as "Stellite 21" (or Vitallium) and "S-816" which contain large amounts of at least one strategically scarce element.

| Alloy         | At 1350° F.                             |                                           | At 1500° F.                             |                                           |
|---------------|-----------------------------------------|-------------------------------------------|-----------------------------------------|-------------------------------------------|
|               | Load (p. s. i.) to fracture in 100 hrs. | Load (p. s. i.) to fracture in 1,000 hrs. | Load (p. s. i.) to fracture in 100 hrs. | Load (p. s. i.) to fracture in 1,000 hrs. |
| Present Alloy | 41,000                                  | 32,000                                    | 24,000                                  | 16,000                                    |
| "Stellite 21" | 34,000                                  | 21,000                                    | 22,000                                  | 14,000                                    |
| "S-816"       | 40,000                                  | 29,000                                    | 26,000                                  | 21,000                                    |

In making the foregoing comparison, the alloy of the present invention had a composition of about 35% nickel, 28% chromium, 9% molybdenum, 0.15% boron, 1.0% carbon, 1.5% manganese, 0.5% silicon and the balance essentially iron. The alloy referred to in the prior art as "Stellite 21" contained about 2% nickel, 27% chromium, 6% molybdenum, 0.25% carbon, 0.6% manganese, 0.6% silicon and the balance cobalt, while the prior art alloy referred to as "S-816" contained about 20% nickel, 18% chromium, 4% tungsten, 4% columbium, 4% molybdenum, 0.4% carbon, 0.6% manganese, 0.3% silicon and the balance cobalt. As illustrative of the temperature range over which the aforementioned composition of the present alloy exhibits good 100-hour and 1000-hour rupture strengths, attention is directed to Fig. 2 which depicts the rupture strengths of the alloy at temperatures from about 1300° F. up to about 1800° F.

A further illustration of the high rupture properties which can be obtained without the use of strategically scarce elements by compositions within the preferred range at various high temperatures is shown graphically in Fig. 3 which depicts stress rupture curves obtained as a result of many tests at temperatures of 1350° F., 1500° F., 1650° F., and 1800° F. The alloys employed in the tests ranged in composition from about 33.8% to 35.4% nickel, about 26% to 28% chromium, about 8% to 9% molybdenum, about 0.86% to 1.06% carbon, about 0.1% to 0.25% boron, about 1.5% to 2% manganese, about 0.3% to 0.5% silicon and the balance essentially iron plus incidental elements.

The improved properties of the cast alloy provided by the invention, which are obtained when the three aforementioned elements molybdenum, boron and carbon are properly employed in the alloy, appear to be associated with a type of metallographic structure which

## 11

is different from that normally obtained in the usual heat resisting cast alloy. The metallographic structure of the present alloy in the as-cast condition comprises a matrix of structureless austenite, containing massive, primary carbide as an almost continuous interdendritic phase with portions of the carbide having a eutectiferous structure.

The high properties which are provided by the relatively non-strategic novel alloy contemplated by the present invention are obtained in the as-cast condition without resorting to the usual high temperature heat treatments, age-hardening treatments, etc. However, if it is desired to improve the room temperature ductility of the alloy provided by the invention, the alloy can be subjected to a high temperature heating comprising heating the cast alloy to a temperature range of about 1900° F. to about 2250° F. for a period of the order of about one-half to one hour or more followed by a normal rate of cooling similar to that obtained when cooling in air.

Properties of the alloy provided by the invention useful in designing articles made thereof include the tensile strength at room temperature and at elevated temperatures and the mean coefficient of expansion. The alloy exhibits a tensile strength of about 70,000 p. s. i. at room temperature and about 60,000 p. s. i. at 1500° F. The mean coefficient of expansion (inch/inch/° F.) of the alloy over various temperature ranges from room temperature up to 1800° F. is as follows:

| From Room Temperature to— | Mean Coefficient     |
|---------------------------|----------------------|
| 500° F.                   | $7.3 \times 10^{-6}$ |
| 1000° F.                  | $8.1 \times 10^{-6}$ |
| 1350° F.                  | $8.5 \times 10^{-6}$ |
| 1500° F.                  | $8.6 \times 10^{-6}$ |
| 1800° F.                  | $8.9 \times 10^{-6}$ |

While the novel alloy provided by the invention is particularly adaptable to the manufacture of articles by precision casting, it is to be understood that the articles made thereof may be produced by other methods, such as other casting methods, powder metallurgy, etc.

The present invention is particularly applicable to the fabrication of cast articles, e. g., blading material, for use in power units of turbine engines, turbojet engines, and the like, and also applicable to the fabrication of articles by other conventional methods of casting for use at elevated temperatures under conditions where a high degree of resistance to deformation under stress is required. Some of the articles which can be made from the alloy provided by the invention include turbine blades for use as rotary and stationary blades, i. e., turbine buckets and nozzle vanes, etc.

Although the present invention has been described in conjunction with preferred embodiments, it is to be understood that modifications and variations may be resorted to without departing from the spirit and scope of the invention, as those skilled in the art will readily understand. Such modifications and variations are considered to be within the purview and scope of the invention and appended claims.

I claim:

1. A substantially cobalt-free, columbium-free, tungsten-free, nickel-chromium-iron precision cast article of manufacture suitable for use at high temperatures in power plant units of gas turbines, turbojet engines and the like, said cast article being comprised of a precision cast alloy characterized by a 100-hour rupture stress at 1350° F. of at least about 37,000 p. s. i. and containing about 30% to 34% nickel, 23% to 27% chromium, 8% to 10% molybdenum, 0.05% to 0.3% boron, 0.6% to 1% carbon, 0.1% to 2% silicon, 0.1% to 3% manganese and the balance except for small amounts of other ele-

## 12

ments which do not materially adversely affect the novel and basic characteristics of the alloy.

2. A substantially cobalt-free, columbium-free, tungsten-free, nickel-chromium-iron precision cast article of manufacture suitable for use at high temperatures in power plant units of gas turbines, turbojet engines and the like, said cast article being comprised of a precision cast alloy characterized by a 100-hour rupture stress at 1350° F. of at least about 37,000 p. s. i. and containing about 20% to 40% nickel, 20% to 30% chromium, 8% to 10% molybdenum, 0.10 to 0.3% boron, 0.6% to 1.2% carbon, 0.1% to 2% silicon, 0.1% to 3% manganese and the balance iron except for small amounts of other elements which do not materially adversely affect the novel and basic characteristics of the alloy, the iron content constituting about 15% to 50% of the alloy.

3. A cobalt-free, columbium-free, tungsten-free, nickel-chromium-iron precision cast article of manufacture suitable for use at high temperatures in power plant units of gas turbines, turbojet engines and the like, said precision cast article being comprised of an alloy characterized by improved 100-hour rupture stress at 1350° F. and containing about 20% to 40% nickel, 20% to 30% chromium, 8% to 10% molybdenum, 0.05% to 0.3% boron, 0.6% to 1.2% carbon, 0.1% to 2% silicon, 0.1% to 3% manganese and the balance iron except for small amounts of other elements which do not materially adversely affect the novel and basic characteristics of the alloy, the iron content constituting about 15% to 50% of the alloy.

4. A substantially cobalt-free, columbium-free, tungsten-free, nickel-chromium-iron precision cast article of manufacture suitable for use at high temperatures in power plant units of gas turbines, turbojet engines and the like, said precision cast article being comprised of an alloy characterized by improved 100-hour rupture stress at 1350° F. and containing about 19% to 50% nickel, 18% to 30% chromium, 8% to 12% molybdenum, 0.03% to 0.8% boron, 0.5% to 1.5% carbon, up to 2% silicon, up to 3% manganese and the balance iron except for small amounts of other elements which do not materially adversely affect the novel and basic characteristics of the alloy, the iron content constituting about 10% to 55% of the alloy.

5. A cobalt-free, columbium-free, tungsten-free, nickel-chromium-iron casting alloy suitable for use at high temperatures in power plant units of gas turbines, turbojet engines and the like, said casting alloy being characterized by improved 100-hour rupture stress at 1350° F. and being comprised of about 30% to 34% nickel, 23% to 27% chromium, 8% to 10% molybdenum, 0.05% to 0.3% boron, 0.6% to 1% carbon and the balance iron except for small amounts of other elements which do not materially adversely affect the novel and basic characteristics of the alloy.

6. A cobalt-free, columbium-free, tungsten-free, nickel-chromium-iron casting alloy suitable for use at high temperatures in power plant units of gas turbines, turbojet engines and the like, said casting alloy being characterized by improved 100-hour rupture stress at 1350° F. and being comprised of about 20% to 40% nickel, 20% to 30% chromium, 8% to 10% molybdenum, 0.10% to 0.3% boron, 0.6% to 1.2% carbon and the balance iron except for small amounts of other elements which do not materially adversely affect the novel and basic characteristics of the alloy, the iron content constituting about 15% to 50% of the alloy.

7. A substantially cobalt-free, columbium-free, tungsten-free, nickel-chromium-iron casting alloy suitable for use at elevated temperatures in power plant units of gas turbines, turbojet engines and the like, said casting alloy being characterized by improved 100-hour rupture stress at 1350° F. and being comprised of about 20% to 40% nickel, 20% to 30% chromium, 8% to 10% molybdenum, 0.05% to 0.3% boron, 0.6%

to 1.2% carbon and the balance iron except for small amounts of other elements which do not materially adversely affect the novel and basic characteristics of the alloy, the iron content constituting about 15% to 50% of the alloy.

8. A substantially cobalt-free, columbium-free, tungsten-free, nickel-chromium-iron alloy suitable for use at elevated temperatures in power plant units of gas turbines, turbojet engines and the like, said alloy being characterized by improved 100-hour rupture stress at 1350° F. and being comprised of about 19% to 50% nickel, 18% to 30% chromium, 8% to 12% molybdenum, 0.10% to 0.3% boron, 0.5% to 1.5% carbon and the balance iron except for small amounts of other elements which do not materially adversely affect the novel and basic characteristics of the alloy, the iron content constituting at least about 10% of the alloy.

9. A substantially cobalt-free, columbium-free, tung-

sten-free, nickel-chromium-iron alloy suitable for use at elevated temperatures in power plant units of gas turbines, turbojet engines and the like, said alloy being characterized by improved 100-hour rupture stress at 1350° F. and being comprised of about 19% to 50% nickel, 18% to 30% chromium, 8% to 12% molybdenum, 0.03% to 0.8% boron, 0.5% to 1.5% carbon and the balance iron except for small amounts of other elements which do not materially adversely affect the novel and basic characteristics of the alloy, the iron content constituting at least about 10% of the alloy.

#### References Cited in the file of this patent

##### UNITED STATES PATENTS

|           |                     |               |
|-----------|---------------------|---------------|
| 2,403,128 | Scott et al. -----  | July 2, 1946  |
| 2,513,472 | Franks et al. ----- | July 4, 1950  |
| 2,562,854 | Binder -----        | July 31, 1951 |